

Aug. 12, 1958

J. A. GESHNER

2,847,333

METHODS OF MAKING MAGNETIC CORES

Filed July 10, 1956

2 Sheets-Sheet 1



FIG. 1



FIG. 2

INVENTOR.  
BY J. A. GESHNER  
Q. C. Schwartz, Jr.  
ATTORNEY

Aug. 12, 1958

J. A. GESHNER

2,847,333

METHODS OF MAKING MAGNETIC CORES

Filed July 10, 1956

2 Sheets-Sheet 2



F/G. 5



F/G. 4



F/G. 3

INVENTOR.

J. A. GESHNER

BY  
A. C. Schwartz, Jr.  
ATTORNEY

## METHODS OF MAKING MAGNETIC CORES

John Allen Geshner, Downers Grove, Ill., assignor to Western Electric Company, Incorporated, New York, N.Y., a corporation of New York

Application July 10, 1956, Serial No. 596,866

8 Claims. (Cl. 117—232)

This invention relates to methods of making magnetic cores, and in particular to methods of making stabilized magnetic cores of the compressed dust type.

One type of inductive loading coil used extensively in the communications field includes a generally toroidal-shaped magnetic core and a wire winding thereon. The magnetic core comprises finely divided particles of a magnetic material. The particles are coated individually with a combination insulator and binder material, and then are compressed into a core body of the desired shape. Before such magnetic cores are provided with their wire windings, a protective coating may be applied to the surfaces of the magnetic cores, which is designed to provide a high degree of both mechanical and electrical protection.

In the manufacture of loading coils of this type, it is desirable to control the temperature stability of inductance of the finished coils. A conventional test for the temperature stability of inductance involves placing a sample coil in a desiccator and subjecting the coil to various temperatures for prolonged periods of time, while simultaneously taking inductance measurements at periodic intervals. The inductance of the sample coil with varying temperatures and time is observed, and the percentage change in the inductance from zero to a maximum change is considered to be the stability coefficient of the particular batch from which the sample loading coil was taken.

More specifically a standard test of this type involves placing the sample coil in a desiccator for twenty hours at a temperature of approximately 30° F., followed by about twenty hours more at a temperature of approximately 130° F., after which the temperature is reduced to 30° F. Measurements of the inductance of the sample coil are recorded throughout the test and compared with the measured value of inductance of the sample coil before the start of the test, whereby there is obtained the stability coefficient of the particular batch from which the sample coil was taken. Although it is desirable that the stability coefficient be zero, finished loading coils having stability coefficients within the range of  $\pm 0.1\%$  are acceptable in the manufacture of loading coils having molybdenum-permalloy powder magnetic cores.

The stability coefficient of uncoated coils is found generally to be of the order of from about  $+0.5\%$  to about  $+1.0\%$ . To reduce the stability coefficient to within the desired tolerance of  $\pm 0.1\%$ , it has been the practice to add to the molybdenum-permalloy dust from which the magnetic cores are formed a sufficient quantity of a low Curie point "stabilizer" dust, having a negative stability coefficient, to reduce the stability coefficient of the finished loading coils to within the desired range. It would be advantageous if the desired stability coefficient of a finished loading coil could be obtained in some other manner.

It is an object of this invention to provide new and improved methods of making magnetic cores.

Another object of this invention is to provide new and improved methods of making stabilized magnetic cores of the compressed dust type.

5 A method of making magnetic cores illustrating certain features of the invention may include the steps of forming such a core from a magnetic material having characteristics such that the formed core has a positive temperature stability of inductance coefficient, and covering the magnetic core with at least one coating of a material having a negative stability effect sufficient to reduce the positive temperature stability of inductance coefficient of the core.

10 A complete understanding of the invention may be obtained from the following detailed description of methods forming specific embodiments thereof, when read in conjunction with appended drawings, in which:

15 Fig. 1 illustrates a magnetic core of the compressed dust type having its electrical characteristics stabilized in accordance with the present invention;

20 Fig. 2 is an enlarged, fragmentary vertical section of the magnetic core shown in Fig. 1;

25 Fig. 3 is a graph illustrating the percentage inductance variation with time and temperature for a typical loading coil having an uncoated magnetic core;

30 Fig. 4 is a graph illustrating the percentage inductance variation with time and temperature for a loading coil with a magnetic core formed from the same batch of alloy dust as the last-mentioned magnetic core, but having several layers of an organic finish, and

35 Fig. 5 is a graph illustrating the percentage inductance variation with time and temperature for a loading coil with a magnetic core formed from the above-mentioned batch of alloy dust, but having a greater predetermined number of layers of the organic finish.

40 The present invention is designed primarily for the stabilization of electrical properties of molybdenum-permalloy dust magnetic cores. In carrying out the present invention a large number of magnetic cores are fabricated by a conventional process from a common batch

45 of insulated alloy dust which is placed in molds and compressed into generally toroidal-shaped magnetic cores of identical dimensions. A sample magnetic core is selected at random and provided with a wire winding of a predetermined number of turns.

45 The wound magnetic core is then placed in a desiccator and subjected to a temperature stability of inductance test of the type described hereinabove. During this test inductance measurements are made periodically to determine the stability coefficient of the magnetic cores without a protective surface coating.

50 Illustrated in Fig. 3 is a graph of the results of such a temperature stability test performed on a typical magnetic core without a surface coating. From Fig. 3 it may be seen that the sample magnetic core so tested has a stability coefficient of approximately  $+0.57\%$ , which is not within the allowable tolerance of  $\pm 0.1\%$ . This value of  $+0.57\%$  may be taken as the stability coefficient for the entire group of magnetic cores fabricated from the particular common batch of insulated alloy dust.

55 In accordance with this invention, the positive stability coefficient of this particular group of magnetic cores may be reduced to within the desired tolerance of  $\pm 0.1\%$  by applying successive coatings of one or more pigmented or unpigmented organic finishes, such as clear varnish,

60 pigmented varnish, enamels or the like, to the surfaces of the magnetic cores. The individual coatings of the organic finishes preferably are applied by spraying, but may be produced otherwise by conventional methods, such as dipping or the like. Each individual coating of an organic finish is dried and baked before the application of the next successive coating. The drying and bak-

3

ing may be accomplished by an initial air drying period followed by a period of baking at an elevated temperature of the order of 350° F. The air drying period should be sufficiently long to prevent blistering during the subsequent baking operation. It is desirable that each of the individual coatings of finish so formed be impervious and have a minimum thickness of approximately .0004 inch.

It has been found that coatings of certain organic finishes have a negative stability coefficient effect and, that, by applying a predetermined number of successive coatings of such organic finishes to a magnetic core fabricated from a given batch of insulated alloy dust, a finished coil having a stability coefficient within the acceptable tolerance of  $\pm 0.1\%$  may be produced. Successive coatings of such organic finishes have an accumulative effect, that is, the predetermined negative stability coefficient effect of one coating adds to the predetermined negative stability coefficient effect of other coatings to produce a greater negative stability coefficient effect.

To determine the number of layers of a given organic finish or finishes required to achieve a stability coefficient of  $\pm 0.1\%$  for a particular group of coils having magnetic cores fabricated from the same batch of insulated alloy dust, sample magnetic cores are tested in accordance with the previously described test procedures for temperature stability of inductance. Once the number of layers of such organic finishes required to produce a finished coil having a stability coefficient of  $\pm 0.1\%$  is determined, all of the other magnetic cores are provided with an equal number of coatings in the same manner to achieve similar results.

The following examples illustrate the invention. These examples are given only for the purpose of illustration and are not intended to limit the invention.

### *Example 1*

A sample magnetic core selected at random from a large number of substantially identical magnetic cores fabricated from a common batch of insulated alloy dust was tested in the manner previously described and found to have a stability coefficient of  $\pm 0.57\%$  as shown in Fig. 3. Another magnetic core selected at random from the same group was provided with three successive, individual coatings of an unpigmented insulating varnish of substantially the following composition.

| Material                                                                                 | Percent By Weight of the Varnish |
|------------------------------------------------------------------------------------------|----------------------------------|
| Heat reactive, oil soluble varnish resin (butyl phenol formaldehyde, alkaline catalyzed) | 4                                |
| Industrial xylene                                                                        | 5                                |

A varnish resin of the type described above may be obtained commercially as BR-10282 alkali refined linseed oil varnish manufactured by Bakelite Company, New York city, N. Y.

Each coating of the varnish was sprayed on the core, was suitably air dried and then baked by infra-red heating at a temperature of approximately 350° F. Each coating of the varnish had a minimum thickness of approximately 0.0004 and a maximum thickness of approximately 0.0007 inch, and was substantially free from blisters or like imperfections.

The sample magnetic core having three coatings of the varnish was tested for its temperature stability of inductance in the manner previously described. The results of this test are illustrated graphically in Fig. 4. It may be seen from Fig. 4 that three successive coatings of the varnish had a negative stability effect sufficient to reduce the stability coefficient to  $\pm 0.17\%$ . However, a sta-

4

ability coefficient of  $+0.17\%$  is still not within the acceptable tolerance of  $\pm 0.1\%$ .

Another magnetic core was selected from the same group of unfinished magnetic cores and eight successive 5 coatings of the same insulating varnish were applied in the manner hereinabove described. The magnetic core having eight coatings of the varnish finish, when subjected to the temperature stability of inductance test, was found to have a stability coefficient of  $+0.1\%$ . The results of 10 the latter test are illustrated graphically in Fig. 5. Accordingly, all of the remaining magnetic cores fabricated from the common batch of insulated alloy can be treated in a like manner (i. e. provided with a minimum of eight 15 coatings of the varnish finish) to produce finished loading coils having stability coefficients within the acceptable tolerance of  $+0.1\%$ .

The application of additional coatings of the varnish finish further decreases the stability coefficient and, if a sufficient number of coatings of the varnish finish are applied, the stability coefficient will become negative and may even fall without the negative stability coefficient limit of  $-0.1\%$ . For example, the application of twenty coatings of the varnish finish produced a coil having a stability coefficient of  $-0.19\%$ .

### *Example II*

A sample magnetic core initially having a stability coefficient of +0.57%, as shown in Fig. 3, was provided with four coatings of the unpigmented insulating varnish heretofore described in connection with Example I. The thus coated core was given an additional single coating of a pigmented insulating varnish having the following composition:

| Material                                                                                 | Percent by Weight of the Varnish |
|------------------------------------------------------------------------------------------|----------------------------------|
| Heat reactive, oil soluble varnish resin (butyl phenol formaldehyde, alkaline catalyzed) | 32                               |
| Industrial xylene                                                                        | 36                               |
| Titanium dioxide                                                                         | 32                               |

A varnish resin of the type described above may be obtained commercially as BR-10282 alkali refined linseed oil varnish manufactured by Bakelite Company, New York city, N. Y.

50 The individual coatings of unpigmented insulating varnish and pigmented insulating varnish were applied in the same manner described in connection with Example I. The magnetic core having four coatings of unpigmented insulating varnish and one layer of pigmented insulating 55 varnish was tested for temperature stability of inductance and was found to have a stability coefficient of  $+0.05\%$ . Thus it may be seen that the layer of pigmented insulating varnish has a somewhat greater negative stability effect than a coating of the unpigmented insulating varnish.

*Example III*

As further evidence of this phenomenon, a magnetic core initially having a stability coefficient of +0.57% was provided with two coatings of the unpigmented insulating varnish described previously in Example I. Three coatings of the pigmented insulating varnish described in Example II were then applied, and the resulting coated core was found to possess a stability coefficient of +0.10%.

70 — 0.19%. It will be understood that this invention is not limited to the specific organic finishes mentioned, namely unpigmented insulating varnish and pigmented insulating varnish. Other suitable pigmented or unpigmented organic finishes having negative stability characteristics

include enamels, such as a white baking enamel having the following composition:

| Material                                                                                                                  | Percent by Weight of the Enamel |
|---------------------------------------------------------------------------------------------------------------------------|---------------------------------|
| Titanium dioxide.....                                                                                                     | 30.9                            |
| Dehydrated castor oil or linseed oil modified glyceryl phthalate alkyd resin containing 38 to 45% phthalic anhydride..... | 30.4                            |
| Industrial xylene.....                                                                                                    | 30.4                            |
| Aromatic solvent (petroleum or coal tar; distillation range 150 to 250°C).....                                            | 8.3                             |

Further, it will be understood that this invention is not limited to any specific number of coatings of such material nor is it intended to limit the thickness of such coatings to any specific dimension.

It is manifest that principles of the invention have manifold applications and that the invention is not limited to the specific examples described hereinabove.

What is claimed is:

1. The method of making temperature stabilized magnetic cores, which comprises forming a core from a magnetic material having characteristics such that the formed core has a positive temperature stability of inductance coefficient, and covering the core with at least one coating of a material having a negative stability characteristic sufficient to reduce the positive temperature stability of inductance coefficient of the core.

2. The method of making temperature stabilized magnetic cores, which comprises forming a core from a magnetic material having a positive temperature stability of inductance coefficient, and applying a plurality of coatings of a material having a negative stability characteristic to reduce the positive temperature stability of inductance coefficient of the core.

3. The method of making temperature stabilized magnetic cores, which comprises forming a core from a magnetic material having a positive temperature stability of inductance coefficient, and coating the core with a material having a negative stability characteristic until the thus coated core has a substantially zero temperature stability of inductance coefficient.

4. The method of making temperature stabilized magnetic cores, which comprises forming a core from a magnetic material having a positive temperature stability of inductance coefficient, and applying coatings of a material having a negative stability characteristic until

the thus coated core has a substantially zero temperature stability of inductance coefficient.

5. The method of making temperature stabilized magnetic cores, which comprises forming a core from a magnetic material having a positive temperature stability of inductance coefficient, and applying to the surface of the core a plurality of layers of an organic finish having a negative stability characteristic until the finished coated core has a temperature stability of inductance coefficient substantially less than that of the uncoated magnetic core.

6. The method of making temperature stabilized magnetic cores, which comprises forming a core from a magnetic material having a positive temperature stability of inductance coefficient, and applying to the surface of the core a number of layers of a varnish having a negative stability characteristic, the number of layers being sufficient to reduce the temperature stability of inductance coefficient of the coated core to substantially less than that of the uncoated magnetic core.

7. The method of making temperature stabilized magnetic cores, which comprises forming a core from a magnetic material having a positive temperature stability of inductance coefficient, and applying to the surface of the core a plurality of layers of an enamel having a negative stability characteristic, the number of layers being sufficient to produce in the finished coated core a substantially zero temperature stability of inductance coefficient.

8. The method of making temperature stabilized magnetic cores of the compressed dust type, which comprises forming a core from a dust-like magnetic material having a positive temperature stability of inductance coefficient, and applying to the surface of the core a sufficient number of layers of pigmented and unpigmented varnish having a negative stability effect to produce in the finished coated core a temperature stability of inductance coefficient substantially less than that of the uncoated magnetic core.

40

#### References Cited in the file of this patent

#### UNITED STATES PATENTS

|           |                |               |
|-----------|----------------|---------------|
| 434,164   | Terry          | Aug. 12, 1890 |
| 2,059,441 | Converse       | Nov. 3, 1937  |
| 2,076,230 | Gillis         | Apr. 6, 1937  |
| 2,307,588 | Jackson et al. | June 5, 1943  |

45